

# UNITED STATES PATENT OFFICE.

CLARENCE R. ECKERT, OF CHICAGO, ILLINOIS, ASSIGNOR TO THE BARRETT COMPANY,  
OF NEW YORK, N. Y., A CORPORATION OF WEST VIRGINIA.

## METHOD OF MANUFACTURING COKE FROM PITCH AND THE PRODUCT THEREOF.

1,213,763.

Specification of Letters Patent.

Patented Jan. 23, 1917.

No Drawing.

Application filed September 10, 1915. Serial No. 49,901.

To all whom it may concern:

Be it known that I, CLARENCE R. ECKERT, a citizen of the United States, residing in the city of Chicago, county of Cook, and State of Illinois, have invented new and useful Improvements in Methods of Manufacturing Coke from Pitch and the Products Thereof, of which the following is a specification.

10 My invention consists in a new method of coking coal tar pitches, and the product thereof, as hereinafter described and claimed.

In the treating of pitch, either hard coal tar pitch, water gas tar pitch, or asphalt, by itself in a coking oven, serious difficulty is encountered because the material, or a portion of it, on reaching a critical temperature varying with the particular material used, suddenly decomposes with large evolution of vapors resulting in sudden and considerable foaming. The expansion of volume caused by this foaming is so great that it is ordinarily impossible to charge 25 the oven with pitch to more than about one-half the capacity of the oven for coking coal. Hence it is obvious that if pitch can be so treated as to prevent foaming in the coking process without material deterioration in the quality of the product, the coke ovens can be operated much more efficiently and economically.

I have found, by extended experimental tests and commercial operations, that with 35 the addition to the pitch of a very small proportion of what is known as coke "breeze," viz: small fragments of ordinary or metallurgical coke, the mixture can be coked practically without any foaming, so as to enable the oven to be charged to approximately full capacity. A workable and practical proportion of such mixture I have found to be about 90% of pitch and 10% of coke breeze. Although such breeze has a 45 larger percentage of ash than pitch, yet the small percentage of breeze does not materially increase the amount of ash in the product over that of a coke manufactured from pitch alone. For example, pitch of the character described ordinarily contains less than .5% of ash. Assuming that the coke breeze has a percentage of 14% of ash, the ash present in the mixture of 90% pitch with 10% breeze would be about

1.85%, which may be considered as negligible, and a coke from the mixed materials is for most practical purposes as valuable as if made from pitch alone. The admixture of coke breeze with pitch may be accomplished in various ways, but I prefer to first grind the pitch so as to pass through a screen of  $\frac{3}{8}$ " mesh, and then mix the breeze therewith while cold. The mixture is then placed in a coke oven of any proper type, or gas retort, and heated in the usual manner to such temperature, and for such period of time, as is necessary to drive off substantially all of the volatile matter. I may, however, mix the coke breeze with pitch, while the latter is in a melted liquid condition, or I may bring the two together in any convenient manner, either before or after introducing them to the coke oven or coking chamber.

Where I use the term "coke oven" I refer particularly to the usual type of by-product coke oven, but I may use any other type of oven suitable for the purpose in hand. For example, I may coke my mixture in gas retorts, either of horizontal, inclined, or vertical type, or in coke ovens not equipped for recovery of by-products, but inasmuch as valuable by-products can be recovered from the coking operation according to my invention, I would ordinarily employ a type of oven suitable for such recovery.

Where I use the term "hydrocarbon" in this specification and in the claims, I refer to such a material as coal tar pitch or its equivalent. For example, I may use either a soft or a hard grade of coal tar pitch, or I may use water gas tar pitch, or oil tar pitch, or petroleum pitch, or asphalt, or any equivalent material. All of these hydrocarbons are characterized by being practically free from ash, usually less than 0.5% of ash. This freedom from ash in the hydrocarbons offsets the relatively higher percentage of ash in the coke breeze and gives a coked product relatively low in ash.

Instead of using coke breeze to mix with the pitch, I may employ other solid carbonaceous material which is non-liquefiable by heat, such for example, as sawdust, charcoal, coal, or like products capable of substitution therefor.

Having thus described my invention,

what I claim and desire to secure by Letters Patent is:

1. The process of manufacturing coke from coal tar pitch or similar hydrocarbons, which consists in mixing therewith a sufficient amount only of solid carbonaceous material non-liquefiable by heat to practically prevent foaming of the hydrocarbon at critical heat and then subjecting the mixture to the coking operation. 35
2. In the manufacture of coke from pitch and similar hydrocarbons, the method, which consists in mixing with the hydrocarbon coke breeze in substantially the proportions of 90% of hydrocarbon and 10% of coke breeze, and afterward subjecting the mixture to a coking operation. 40
3. In the manufacture of coke pitch, the method, which consists in mixing with pitch, coke breeze in substantially the proportions of 90% of pitch to 10% of breeze. 45
4. In the manufacture of coke from pitch and similar hydrocarbons, the method which consists in mixing with the pitch solid carbonaceous material in substantially the proportions of 90% of pitch and 10% of the solid carbonaceous material, and afterward subjecting the mixture to a coking operation. 50
5. In the manufacture of coke from coal 55

tar pitch and similar hydrocarbons, the method of adding to the pitch a sufficient amount of solid carbonaceous material non-liquefiable by heat to substantially prevent the foaming of the hydrocarbon.

6. In the manufacture of coke from coal tar pitch and similar hydrocarbons, the method of preventing foaming of the hydrocarbon at the critical temperature, which consists in mixing with the hydrocarbon a sufficient amount of solid carbonaceous material non-liquefiable by heat as will substantially prevent the foaming of the hydrocarbon. 40

7. As a new product, coke manufactured from a mixture of about 90% of hydrocarbon and 10% of solid carbonaceous material non-liquefiable by heat. 45

8. As a new product, a coke manufactured from a mixture of pitch and solid carbonaceous material and containing not to exceed 3% of ash. 50

9. As a new product, a coke manufactured from a mixture of pitch and coke breeze and containing not to exceed 3% of ash. 55

Signed at Chicago in the county of Cook and State of Illinois, this 3rd day of September, 1915.

CLARENCE R. ECKERT.